

[54] PHOTOGRAPHIC FILM WITH  
POLYETHYLENE  
TEREPHTHALATE-POLYALKYLENE  
GLYCOL COPOLYMER SUPPORT[75] Inventors: Kenji Yabe; Atsuhiko Soda, both of  
Otsu; Satoyuki Minami; Osamu Iida,  
both of Mishima, all of Japan[73] Assignees: Fuji Photo Film Co., Ltd.,  
Minami-ashigara; Toray Industries  
Inc., Nihonbashimuro, both of Japan

[21] Appl. No.: 876,800

[22] Filed: Feb. 10, 1978

## [30] Foreign Application Priority Data

Feb. 10, 1977 [JP] Japan ..... 52-12931

[51] Int. Cl.<sup>2</sup> ..... G03C 7/00; G03C 1/40;  
G03C 1/78; G03C 1/96[52] U.S. Cl. ..... 430/211; 430/533;  
525/227; 428/480[58] Field of Search ..... 96/76 R, 76 C, 77, 87 R,  
96/3, 29 D, 73; 428/480; 260/860

## [56] References Cited

## U.S. PATENT DOCUMENTS

3,635,707 1/1972 Cole ..... 96/77  
3,988,157 10/1976 Van Paesschen et al. ..... 96/87 RPrimary Examiner—Richard L. Schilling  
Attorney, Agent, or Firm—Sughrue, Rothwell, Mion,  
Zinn and Macpeak

## [57] ABSTRACT

A diffusion transfer photographic film, in which a film of a polyethylene terephthalate copolymer is a part of the constituents thereof, the polyethylene terephthalate containing about 3 to about 20% by weight of a polyalkylene glycol, as a glycol component comonomer, based on the weight of the polyethylene terephthalate copolymer.

31 Claims, 3 Drawing Figures



**FIG 1****FIG 2****FIG 3**

PHOTOGRAPHIC FILM WITH POLYETHYLENE  
TEREPHTHALATE-POLYALKYLENE GLYCOL  
COPOLYMER SUPPORT

BACKGROUND OF THE INVENTION

1. Field of the Invention

This invention relates to a diffusion transfer photographic film which provides an excellent print and which has excellent dimensional stability.

2. Description of the Prior Art

Recently, diffusion transfer photography enabling photographed pictures to be viewed on the spot has spread increasingly due to its convenience.

The structure of diffusion transfer photographic films, in particular, the structure of diffusion transfer color photographic films, more or less varies dependent upon the processes for developing and printing them as described in, for example, *Properties of Films and Processing Arts Therefor* (published by Shashin Kogyo Shuppan Sha, Oct. 15, 1976). In principle, however, the photographic film comprises the constituents necessary for photography, development and printing.

A detailed description and explanation of diffusion transfer photographic films are set forth below.

The so-called diffusion transfer process instant color photographic light-sensitive materials as well known as diffusion transfer photographic films in the photographic art. In these types of materials, diffusible dyes are image-wise released from a light-sensitive element in conformity with the images exposure. Of these materials, film units in which a development processing solution is spread as a thin layer immediately after photographing and which does not require the image-receiving layer to be separated from the light-sensitive element by, e.g., an operation such as delamination, and which permits the composite to be used as a photographic picture are advantageous since they have the advantages that they are handy, their procedure of use is simplified, the development processing solution is not uncovered and, therefore, clothes are not stained by the processing solution, and no waste materials due to delamination are produced. These composite film units are described in U.S. Pat. Nos. 2,983,605, 3,415,645, 3,415,646, 3,415,644, 3,578,540, 3,573,043, 3,615,421, 3,594,164, 3,594,165, 3,620,724, 3,635,707, 3,993,486, British Pat. Nos. 1,269,805, 1,330,524, etc., and are well known.

These composite film units contain, sandwiched between two dimensionally stable supports, light-sensitive silver halide emulsion layers, dye image-providing compounds associated with the silver halide emulsions, an image-receiving layer capable of fixing as an image the diffusible dyes released from the dye image-providing compounds, and a light-reflecting layer which serves as a white background for viewing the image formed in the image-receiving layer. In addition, a container retaining a processing solution is disposed at a given position between the two supports and which is capable of spreading a development-processing solution in a layer state thereon. These constituents are fixed together to form a composite structure. In a preferred embodiment, the film unit has, in sequence from the exposure side, a blue-sensitive silver halide emulsion layer having associated therewith a yellow dye image-providing compound, a green-sensitive silver halide emulsion layer having associated therewith a magenta dye image-providing compound and a red-sensitive silver halide emul-

sion layer having associated therewith a cyan dye image-providing compound between the two supports, with these silver halide emulsion layers being advantageously separated from each other by interlayers. In

5 addition, the film unit advantageously contains a polymer acid layer for neutralizing alkali brought into the element with the processing solution after substantial completion of a dye image, and a neutralization timing layer for controlling the formation of an image and the 10 rate of neutralization. Further, the film unit advantageously has a light-intercepting layer which permits the film unit to be processed in a bright room after the film unit comes out of the camera. Additionally, the supports may have a backing layer thereon. The most preferred film unit structure comprises, in sequence from the exposure side, (A) a transparent support—a polymer acid layer—a neutralization timing layer—an image-receiving layer—(a processing solution layer containing a light-reflecting material)—a protective layer—a blue-sensitive silver halide emulsion layer—a yellow dye image-providing compound layer—an interlayer—a green-sensitive silver halide emulsion layer—a magenta dye image-providing compound layer—an interlayer—a red-sensitive silver halide emulsion layer—a cyan dye image-providing compound layer—a light-intercepting support; or (B) a transparent support—a polymer acid layer—a neutralization timing layer—(a processing solution layer containing a light-intercepting material)—a protective layer—a blue-sensitive silver halide emulsion layer—a yellow dye image-providing compound layer—an interlayer—a green-sensitive silver halide emulsion layer—a magenta dye image-providing compound layer—an interlayer—a red-sensitive silver halide emulsion layer—a cyan dye image-providing compound layer—a light-intercepting layer—a light-reflecting layer—an image-receiving layer—a transparent support. Film unit (A) described above is exposed through the transparent support, with the image formed being viewed through the same support, whereas film unit (B) described above is exposed through the transparent support adjacent the polymer acid layer, with the image formed being viewed through the transparent support adjacent the image-receiving layer.

The film unit constituents provided between the two supports are bound at the periphery thereof to maintain the composite film unit form prior to, during and after development processing and prevent the spread processing solution from oozing out of the unit, and the film unit is preferably constructed so that a definite space exists between the two supports in order to spread the processing solution in a given thickness. Further, the film unit preferably has a pod retaining the processing solution which is fixedly positioned at one end thereof and a reservoir for receiving excess processing solution which is fixedly positioned at the opposite end thereof. Various bonding or fixing techniques can be used. Typical examples include (i) adhering the two supports externally with a binding member which embraces the two supports (outer spacer) and (ii) adhering photographic layers between the two supports using a binding member (inner spacer).

FIGS. 1, 2 and 3 show examples of the structures of diffusion transfer photographic films, particularly of diffusion transfer color photographic composite film units. In these figures, the details of emulsion layers, although important in the photographic film, are not

shown since they are not necessary to describe the invention, and as a result, these figures illustrate diagrammatic views mainly showing the elements necessary for describing the materials to which the present invention is applicable.

FIG. 1 shows a photographic film of type (A) described above in which the exposure side (A-1) and the print-viewing side (A-2) are on the same side, and FIG. 2 is an enlarged view thereof. In this type of film, transparent film support (1) is on the surface side and black opaque film support (2) is on the back side, with a border (4) of white contact-bonding tape (3). Pod (6) retaining processing solution (5) is attached to the back surface of the lower side of the image layer. Layers between supports (1) and (2) comprise emulsion layer (7), image-receiving layer (8), neutralizing layer (9) for neutralizing the processing solution and processing solution layer (10) to be formed by processing solution (5) released from pod (6) and spread on the image area, and the like. Another example is a photographic film of the type (B) described above wherein the exposure side (B-1) and the print-viewing side (B-2) are on opposite sides of the film as illustrated in FIG. 3. This type of film comprises transparent film supports (1) at the surface and the back side, neutralizing layer (9), processing solution layer (10) to be formed after photographing by processing solution (5) spread from pod (6), emulsion layer (7), light-intercepting black layer (11) and image-receiving layer (8).

After image-wise exposure, these photographic films are passed between rollers to rupture pod (6) retaining processing solution (5) and to spread processing solution (5) over the image area for conducting development and printing. When the photographic films come out of the camera, they are in a sufficiently dry state to be satisfactorily handled, and a printed image gradually becomes distinct to provide a photographic picture in about 5 to 10 minutes.

However, these convenient diffusion transfer photographic films have the following defects in handling after photographing.

(1) The printed surfaces must be handled with care for about 10 minutes after photographing.

(2) It takes such a long time for the water present in the processing solution or the like to escape as a vapor into the atmosphere that the photographic pictures do not easily dry. Thus, a long time is required before the image becomes completely stable.

(3) The photographic pictures obtained cannot be stored in a highly humid place due to reason (2) described above, and hence color change, deformation or blocking with other photographic pictures or with album mounts tends to occur during storage.

With the film unit of, in particular, the inner spacer type as hereinbefore described, the processing solution is not spread on the back of the binding member, and hence a difference occurs in that the central areas (image area) of the two supports come into contact with water of the processing solution, whereas the peripheral area (binding member area) does not come into contact with the water of the processing solution. If the supports are made of a material which will swell to a degree above a certain limit when in contact with water, the area which swells is enclosed in a non-swelling frame, resulting in a distortion of the film unit. With a film unit of the outer spacer type (i), a similar distortion can occur when the binding member is swollen only

with difficulty with water and the mechanical strength thereof is larger than a certain limit.

Various techniques have been developed for removing these defects. For example, (1) choosing constituents including emulsion layers and the like of the film so as to minimize the amount of processing solution, and (2) use of a support film having a large water permeability as the surface layer and the back side layer of a photographic film have been suggested. With respect to approach (1) above, a large number of examinations have been made. However, removal of the above-described defects using this approach has not been sufficient. With respect to approach (2), cellulose triacetate films widely used as a support for motion picture film or photographic film have been examined. It is true that a cellulose triacetate film has excellent water permeability and permits water contained in a photographic film to escape as a vapor, but a cellulose triacetate film is not dimensionally stable under high humidity conditions so that the image surface becomes uneven during escape of water damaging the photographic values. Therefore, at present, unavoidably a polyethylene terephthalate film must be used due to its excellent flatness, dimensional stability under high humidity conditions, chemical resistance and transparency despite its unsatisfactory water permeability.

Stabilization of the image has been attempted by rapidly removing the solvent (in many cases water) of the processing solution from the composite film unit. For example, British Pat. No. 1,313,868 describes the use as a support of a polymer layer of cellulose acetate, regenerated cellulose, cross-linked polyvinyl alcohol, or an extremely thin polyester base, a polyester base containing pores permeable to water vapor (the vapor permeability being not less than 100 g/24 hrs·100 in<sup>2</sup>/mil (corresponding to 394 g/24 hr·m<sup>2</sup>/0.1 mm), preferably not less than 300 g/24hrs·100 in<sup>2</sup>/mil (corresponding to 1182 g/24 hr·m<sup>2</sup>/0.1 mm)). However, the polymer supports specifically described above are not satisfactory for use in a composite film unit due to one of the following defects: (1) the swelling when the polymer supports are in contact with water is so large that the film unit form will be affected when a development processing solution is spread; (2) the deficiency in mechanical strength due to the very thin thickness makes it difficult to coat a photographic layer thereon or to uniformly spread the processing solution; (3) the polyester base containing fine pores (e.g., having a size of 23-107  $\mu$ ) is optically opaque, and hence image-wise exposure through such a support or viewing images through such a support is actually difficult. In particular, with a film unit having a structure where swelling with water is restricted by at least one end of the film unit, a dimensional lack of balance will occur between the image area which swells when in contact with water and the end area which does not swell even in contact with water where a weakly hydrophilic support like cellulose acetate as described above is used. In such a case, the film unit will be seriously deformed after spreading the processing solution, and this deformation remains even after the processing solution is dried away to such a degree that the resulting photograph cannot be satisfactorily utilized any more. In addition, supports with insufficient transparency cannot be used for film unit (B) described above which is a particularly preferable type.

## SUMMARY OF THE INVENTION

As a result of various investigations for removing these defects of diffusion transfer photographic films, on examination of support films, it has now been discovered that the use of a polyester film having substantially the same excellent properties as that of a conventional polyethylene terephthalate film in terms of flatness, dimensional stability under high humidity conditions, chemical resistance and transparency and having improved water permeability and film adhesiveness removes the above-described defects, and thus the present invention has been achieved.

That is, the present invention provides a diffusion transfer photographic film, in which a polyester film is used as one of the constituents of the film, with the polyester film comprising a film of a polyethylene terephthalate copolymer containing about 3 to about 20% by weight of a polyalkylene glycol, as a glycol component comonomer, based on the weight of the polyethylene terephthalate copolymer.

## BRIEF DESCRIPTION OF THE DRAWINGS

FIGS. 1, 2 and 3 are cross-sectional views showing the structures of diffusion transfer photographic films. Although actual photographic films comprise multicoated layers for various purposes, base film layers, etc., these figures are only diagrammatic views sufficient to illustrate the present invention.

FIG. 1 shows one example of the structure of a diffusion transfer photographic film, and FIG. 2 shows a part of enlarged view of the photographic film of FIG. 1.

FIG. 3 shows a part of another example, enlarged as in FIG. 2, of a diffusion transfer photographic film.

In these figures, numeral 1 designates a transparent film base, 2 a black and opaque film base, 3 a white contact bonding tape, 4 a border formed by the white contact bonding tape 3, 5 a processing solution necessary for development and printing, 6 a pod retaining the processing solution, 7 an emulsion layer, 8 an image-receiving layer, 9 a neutralizing layer, 10 a processing solution layer spread after photographing, 11 a black light-intercepting layer, A-1, B-1 the exposure side, and A-2, B-2 the print-viewing side.

## DETAILED DESCRIPTION OF THE INVENTION

The phrase "part of the constituents" as used herein means that the polyester film described above is used as a part of or all of one or more constituents where form-maintaining ability is required and is essential such as transparent film bases at the surface and the back side of a photographic film, an opaque black film base to be used as a light-intercepting layer, a bordering for a photographic picture, a spacer between film bases, a support of the photographic film, a base for a coating layer in the photographic film, e.g., an emulsion layer and the like.

The polyester film in accordance with the present invention must have a water vapor permeability and a humidity swelling coefficient within the scope specified in the present invention. Further, polyester films in accordance with the present invention to be used as the constituents which must have a good transparency, must have a haze of not more than about 10% per sheet, preferably not more than 5%. The polyester films referred to in the present invention desirably have a

Young's modulus of not less than about 250 kg/mm<sup>2</sup>, preferably not less than 300 kg/mm<sup>2</sup> (the average of the value of the Young's modulus in the longitudinal direction and the value of the Young's modulus in the transverse direction of the film).

If the water vapor permeability at 60° C. is less than about 10 g/m<sup>2</sup>·24 hr/0.1 mm, water in a photographic film scarcely escapes as a vapor due to the poor water permeability, and hence the photographic pictures do not dry easily and as long as more than 1 month is necessary for the image to become completely stable. On the other hand, if the water vapor permeability at 60° C. is more than about 100 g/m<sup>2</sup>·24 hr/0.1 mm, water escapes as vapor in such a short time that the surface of the photographic picture becomes uneven or deformation of the photographic picture takes place. If the humidity swelling coefficient at 20° C. is less than about  $1.0 \times 10^{-5}/\% \text{ RH}$ , the dimensional change of layers other than the polyester film layer, such as the emulsion layers, than the polyester film layer becomes so much larger than that of the polyester film that the polyester films must be thick in order to maintain the dimensional stability of the photographic pictures. On the other hand, if the humidity swelling coefficient at 20° C. is more than about  $6.0 \times 10^{-5}/\% \text{ RH}$ , the dimensional change of the polyester film itself becomes so large that the photographic picture becomes curved or distorted.

Specific examples of polyester films which can be used in the present invention having the above-described properties are films of polyethylene terephthalate copolymers prepared by copolymerizing terephthalic acid with ethylene glycol and a polyalkylene glycol as glycol component comonomers, with the polyalkylene glycol being present in an amount of about 3 to 20% by weight, preferably 3 to 15% by weight, based on the weight of the polyethylene terephthalate copolymer produced and with the polyalkylene glycol having a molecular weight of about 300 to 30,000, preferably 800 to 20,000. Biaxially oriented films are particularly preferable. Typical examples of the polyalkylene glycols which can be used include those having 2 to 4 carbon atoms in the alkylene moiety such as polyethylene glycol (PEG), polypropylene glycol (PPG), poly(ethylene-propylene) glycol copolymer, polytetramethylene glycol (PTMG), etc.

In this case, if the molecular weight of the polyalkylene glycol used for the copolymerization is less than about 300, the mechanical properties become poor, although there are no problems as to the water vapor permeability and the humidity swelling coefficient. On the other hand, if the molecular weight of the polyalkylene glycol is more than about 30,000, defects occur such as the water permeability is low for the copolymerization amount of the polyalkylene glycol and that transparency is reduced, often resulting in the formation of a milky film. Also, if the amount of the polyalkylene glycol copolymerized is less than about 3% by weight, the water vapor permeability and the humidity swelling coefficient are not improved very much. If the amount copolymerized exceeds about 20% by weight, the equilibrium adsorption moisture content of the polyester is so high and the resulting film is so hygroscopic that the problem of susceptibility to heat and thermal decomposition upon melt-extrusion and the problem of coloration occur. In addition, photographic properties of the film prepared using such a polyester have the defect that, when the film is left in a highly humid area, the film absorbs water from the surrounding atmosphere.

Where PEG is used as the polyalkylene glycol, a PEG having a molecular weight of about 300 to 10,000, in particular 800 to 6,000, is preferred. Where the polyester is to be used as a part where transparency is important, a PEG with a molecular weight of 800 to 2,000 is particularly preferred. A suitable amount of these PEG's copolymerized is about 3 to 15% by weight, particularly preferably 4 to 10% by weight. Where a poly(ethylene-propylene) glycol copolymer is used as the polyalkylene glycol, a preferred molecular weight ranges from about 500 to 30,000, particularly preferably 1,000 to 20,000, and the amount copolymerized ranges from about 3 to 15% by weight, particularly preferably 4 to 10% by weight. Where PTMG is used as the polyalkylene glycol, a preferred molecular weight ranges from about 500 to 2,000, particularly preferably from 800 to 1,500, and a preferred amount copolymerized ranges from about 4 to 18% by weight, particularly preferably 5 to 15% by weight.

Of these polyalkylene glycols, PEG is particularly preferred in copolymerization ratio, water permeability and dimensional stability under high humidity conditions.

The above-described specific examples of polyesters are mainly polyesters comprising, as an acid component, terephthalic acid and, as a glycol component, ethylene glycol and polyalkylene glycol. In the present invention, however, those polyesters which contain, as the acid component, dicarboxylic acids such as aromatic or aliphatic dicarboxylic acids (e.g., isophthalic acid, adipic acid, sebacic acid, etc.) and, as the glycol component, diols such as diethylene glycol, 1,4-butanediol, cyclohexanedimethanol, pentanediol, hexanediol, etc., in amounts of these other dicarboxylic acids and other diols which do not cause a deterioration of film properties intended in the present invention, in particular, a reduction in haze and in the mechanical properties, preferably in a copolymerization amount of less than about 10 mol%, may also be used.

To the copolymer polyesters used in the present invention may be added, if desired, an antioxidant, a lubricant, an antistatic agent, a coloration-preventing agent, a pigment, a dye and a viscosity-adjusting agent. In particular, addition of an antioxidant, in particular, a hindered phenol antioxidant, in an amount of about 0.005 to 0.5% by weight, preferably 0.01 to 0.3% by weight is preferred. For example, "Irganox" 1010 (trade name, produced by Ciba-Geigy Co.) is particularly effective. In addition, where the polyester is to be employed also as a light-intercepting layer, the use of carbon black fine particles in an amount of about 0.1 to 5% by weight, although the amount of carbon black will vary depending upon the film thickness, is effective.

In addition, known polymers can be blended with the polyester to be used in this invention depending on the end-use in an amount which does not detrimentally influence the polyester as a base for photographic films. For example, a modified ester obtained by subjecting polyethylene terephthalate to an ester exchange reaction with diols or polyalkylene glycols such as diethylene glycol, triethylene glycol, polyethylene glycol, etc., can be blended in an amount of about 1 to 10% by weight, preferably 3 to 8% by weight, with the polyester to be used in this invention to enhance water permeability.

The polyester film to be used in the present invention is obtained by biaxially orienting an unoriented film which can be produced using conventional melt-extrusion

processes. More specifically, to illustrate one example of a process for forming a film of the polyester film to be used in the present invention, an unoriented film melt-extruded at about 260° C. to 300° C. is oriented about 2.7 to 3.7 times at about 70° to 100° C. in the longitudinal direction of the film using a roll-type longitudinal orientation machine, and then fed to a tenter to orient the film about 2.7 to 3.7 times at about 80 to 120° C. in the transverse direction. Subsequently, the film so treated is subjected to a heat treatment at about 150° C. to 5° C. below the melting point of the polymer under conditions preventing shrinkage of the film or allowing some shrinkage of the film to prepare a biaxially oriented film.

The thickness of the polyester film to be used in the present invention will vary depending on the part for which it is used but, in general, a suitable thickness is about 25 to 250 $\mu$ , preferably 75 to 150 $\mu$ .

The polyester film to be used in the present invention has the characteristics that, as compared with conventional polyethylene terephthalate films, the adhesiveness of the surface and the adhesiveness with various coating layers such as an emulsion layer are improved.

The present invention is particularly applicable to the diffusion transfer instant color photographic light-sensitive materials described hereinbefore, e.g., for the type (A) and of the type (B) described hereinbefore and as shown in FIGS. 1 to 3.

It has been discovered that the following properties can be imparted to diffusion transfer process instant photographic films by using a polyester base of the present invention having an intermediate water vapor permeability and a low humidity swelling coefficient.

(1) Water brought into the film unit with the spread processing solution is rapidly removed from the film unit. As a result of this drying, migration of excess diffusible dyes after formation of the image is depressed, and the tendency of the white background of photographic pictures to be stained during storage or the tendency of the color image gradation to change due to "post transfer" is minimized.

(2) The degree of discoloration and the degree of fading (during storage in a dark place and upon being struck with light) are low. The reason for this is not fully understood, but it may be attributed to the fact that a dry condition is not conducive to discoloration reactions and fading reactions or the fact that the components in the film unit which accelerate the discoloring and fading reactions are prevented from migrating to the image-receiving layer.

(3) The film unit of the present invention is not distorted and retains a good flatness during processing and storage of images, i.e., during the period where water is present or in a dry state. This property is maintained even when the film unit contains, at an end or ends, a part or parts which do not swell even in contact with water.

(4) Image-wise exposure or image-wise viewing through the film base is possible without substantially affecting the image quality. This enables the production of film unit (B) described above which is a particularly preferred type. This is due to the high transparency of the film base of the present invention.

(5) It has become possible to provide the film base with the necessary mechanical strength (rigidity) for spreading the processing solution as a thin layer. Thus, the processing solution can be uniformly spread. This is due to the high transparency of the film base material,

which results in the ability to employ the necessary thickness for spreading the processing solution.

Various dye image-providing materials heretofore known for diffusion transfer color photographic processes can be used in the film unit of the present invention. Examples include those compounds which undergo a change in diffusibility of the dyes, dye precursors or dye-forming moieties thereof as a result of the oxidation reaction accompanying the development of silver halide, for example, those described in U.S. Pat. Nos. 3,227,550, 3,844,785, 3,620,730, 3,719,489, 2,983,606, 3,928,312, 4,055,428, 3,942,987, 3,954,476, 3,993,638, 4,013,633, British Pat. No. 1,464,104, Japanese Patent Application (OPI) No. 104,343/76, etc. In particular, dye developers of the type described in *Nebblette's Handbook of Photography and Reprography*, 7th Ed., pp. 259-330 (1977) and dye releasers of the type described in *Phot. Sci. Eng.*, 20, 155 (1976) can advantageously be used in the present invention.

Various silver halide emulsions of the types corresponding to dye image-providing materials to be associated therewith can be used in the film unit of the present invention. That is, in order to obtain positive images, negative type emulsions are used for such dye image-providing materials as dye developers, and direct-positive type emulsions, in particular, internal latent image-forming type emulsions as described in U.S. Pat. Nos. 3,317,322, 2,592,250, 3,761,276, 3,761,266 and 3,761,267 are used for dye releaser type image-providing materials. These can be sensitized, color sensitized and stabilized using various known techniques.

A development processing solution capable of developing an exposed silver halide emulsion in a film unit and causing formation and transfer of diffusible dyes is used in the film unit of the present invention. This processing solution is an aqueous solution containing the components necessary to cause these photographic processes to occur. For example, the development processing solution contains an alkali agent, an auxiliary developing agent, a development accelerator, an anti-fogging agent, an antioxidant, etc. In addition, the processing solution may contain a thickening polymer facilitating the spreading of the processing solution in a thin layer such as hydroxyethyl cellulose and carboxymethyl cellulose, an opacifying agent, etc. After exposure, the processing solution is uniformly spread in a liquid thickness of about 30 to 180 $\mu$  in the film unit. The processing solution is advantageously retained in a rupturable container, generally called a pod, and released from the container by a means for spreading the processing solution equipped in a camera such as a pair of juxtaposed pressure-applying rollers. The amount of water brought into a film unit with the processing solution will vary depending upon the composition of the processing solution and the thickness of the solution spread but, roughly speaking, the amount of water ranges from about 25 g/m<sup>2</sup> to about 180 g/m<sup>2</sup>.

A particularly preferred embodiment of this invention is a film unit comprising:

(a) a photosensitive element comprising a transparent support having thereon the following layers in sequence: an image-receiving layer; an alkaline solution-permeable light-reflecting layer; an alkaline solution-permeable opaque layer; a red-sensitive silver halide emulsion layer having a cyan dye image-providing compound associated therewith; an interlayer; a green-sensitive halide emulsion layer having a magenta dye image-providing compound associated therewith; an

interlayer; a red-sensitive silver halide emulsion layer having a yellow dye image-providing compound associated therewith; and a protective layer;

5 (b) a cover sheet superposed on the protective layer of the photosensitive element and comprising a transparent support coated in sequence with a neutralizing layer and a neutralization timing layer; and

10 (c) a rupturable container retaining an aqueous alkaline processing composition and an opacifying agent, the rupturable container being so positioned during the processing of the film unit that a compressive force applied to the rupturable container causes a discharge of the alkaline processing composition between the cover sheet and the protective layer of the photosensitive element.

15 A detailed description of the elements used in this film unit, i.e., photosensitive element, cover sheet, processing composition, rupturable container, is given in U.S. Pat. Nos. 4,056,394 and 4,061,496.

The surface of the film base to be used in the present invention can be advantageously subjected to various processings known in the photographic art in order to strongly adhere the photographic layers to be provided thereon containing a hydrophilic binder, such as processing to render the surface of the film base hydrophilic using an ultraviolet light treatment, a corona discharge treatment, a flame treatment and formation of an adhesive polymer (subbing) layer thereon. This film base advantageously contains a slight amount of a pigment or a dye so as to prevent light-piping through the base when the film unit is withdrawn from the camera. This film base advantageously has a thickness of from about 50 to 250 $\mu$  to provide sufficient mechanical strength to support the photographic layers of the film unit and enable the processing solution to be uniformly spread thereon.

20 The methods of measurement of the characteristics of the polyester film employed in this invention are described in detail below.

#### Water Vapor Permeability

Measured at 40° C. according to JIS Z-0208.

#### Humidity Swelling Coefficient

25 A constant load extensometer (made by Nippon Jidosha Seigyo K.K., Model ITL-2) was placed in a thermostatically and humidistically controlled chamber where the temperatures of such could be changed over a broad range, and a load of 2.5 g/cm width was applied to a sample film (150 mm in length by 10 mm in width). The relative humidity was changed at 20° C. within the range of 40 to 80% RH, and the humidity swelling coefficient was determined from the extension in the length of the film versus humidity. Humidity was measured using an Assmann aspiration psychrometer.

#### Photographic Film

30 Sample photographic films were prepared according to the process described in Japanese Patent Publication No. 16,356/71 and, after photographing, developing and printing, the photographic films were left in an atmosphere of a temperature of 20° C. and a humidity of 65% RH. The reduction in moisture content was determined by the weight loss and the flatness of the image areas and the dimensional change such as distortion of the entire films were observed visually.

35 The following examples are given to illustrate the present invention in greater detail. Unless otherwise

indicated herein, all parts, percents, ratios and the like are by weight.

## EXAMPLE 1

Various polyethylene terephthalate copolymers were prepared by copolymerizing 8.0% by weight of polyethylene glycol (PEG) having a molecular weight of 800-20,000 with terephthalic acid. The copolymers were fed to a 40 mm  $\phi$  extruder and melt-extruded at 280° C. to form films. After longitudinally orienting 3.3

5 10

Film No. 7 required longer than 30 days to become dry and had a poor long-term storability.

## EXAMPLE 2

Polyethylene terephthalate copolymers containing 3, 10, 15 and 20% by weight of PEG with a molecular weight of 1,000 were formed into biaxially oriented films of at thickness of 100 $\mu$  in the same manner as in Example 1. The properties of these films are shown in Table 2 below.

TABLE 2

| Film No. | PEG (wt %) | Copolymerization Amount of | Young's Modulus |                          | Water Vapor Permeability (g/m <sup>2</sup> · 24 hr/0.1 mm) | Humidity Swelling Coefficient ( $\times 10^{-5}$ / % RH) |
|----------|------------|----------------------------|-----------------|--------------------------|------------------------------------------------------------|----------------------------------------------------------|
|          |            |                            | Haze (%)        | MD (kg/mm <sup>2</sup> ) | TD (kg/mm <sup>2</sup> )                                   |                                                          |
| 8        | 3          |                            | 1.9             | 360                      | 385                                                        | 11.0                                                     |
| 9        | 10         |                            | 2.5             | 280                      | 330                                                        | 23.8                                                     |
| 10       | 15         |                            | 4.8             | 253                      | 290                                                        | 38.0                                                     |
| 11*      | 20         |                            | 11.0            | 236                      | 258                                                        | 61.2                                                     |

\*Comparative example

times at 80° C., the films were transversely oriented 3.5 times at 90° C. using a tenter and subjected to heat treatment at 200° C. while preventing shrinkage to prepare biaxially oriented films of a thickness of 100 $\mu$ . For comparison, a biaxially oriented film of a non-copolymerized conventional polyethylene terephthalate film was also prepared. The characteristic properties of each film are tabulated in Table 1 below.

25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 10

## EXAMPLE 3

Carbon black was added in an amount of 1.0% by weight to a polyethylene terephthalate copolymer (intrinsic viscosity: 0.73) containing 15% by weight of PEG with a molecular weight of 1,000, and the copolymer with the carbon black was extruded. Then, the resulting unoriented film was longitudinally oriented 3.3 times at 85° C., and then transversely oriented 3.3 times at 90° C., followed by heat treatment at 210° C. while preventing shrinkage to obtain a biaxially oriented film (No.12) having a thickness of 115 $\mu$  and a light-intercepting property. This film had a Young's modulus of 270 (MD) and 280 kg/mm<sup>2</sup> (TD), a water vapor permeability of 41.3 g/m<sup>2</sup>·24 hr/0.1 mm, and a humidity swelling coefficient of  $3.1 \times 10^{-5}$  /% RH. This Film No.12 was used as film (2) in FIG. 1 and Film No.2 in Example 1 was used as film (1) in FIG. 1 to prepare a photographic film. When this film was tested, moisture escaped as a vapor in about 5 days, leaving a clear photographic picture with good flatness.

## EXAMPLE 4

A polyethylene terephthalate copolymer containing 6% by weight of PEG with a molecular weight of 1,000 was blended in varying amounts with a modified polyester (density: 1.34 g/cm<sup>3</sup> (23° C.); softening point: 125° C.; melt index: 13 g/10 min.) obtained by an ester-exchange reaction with polyethylene glycol and diethylene glycol, and 0.1 wt% of "Irganox" 1010 (made by Ciba-Geigy Co.) was added thereto as an antioxidant, followed by pelletizing to uniformly blend the materials. The resulting blend was melt-extruded at 270° C. to form a film, and the extruded film was longitudinally oriented 3.5 times at 80° C., subsequently transversely oriented 3.5 times at 85° C. using a tenter, followed by heat treatment at 200° C. under 1% relaxation to obtain a biaxially oriented film having a thickness of 75 $\mu$ . Blending with the modified polyester improved water permeability substantially without degrading the transparency.

The properties of the films are shown in Table 3 below.

TABLE 3

| Film No. | Modified Polyester (wt. %) | Haze (%) | Water Vapor Permeability (g/m <sup>2</sup> · 24 hr/0.1 mm) | Humidity Swelling Coefficient ( $\times 10^{-5}$ /% RH) |
|----------|----------------------------|----------|------------------------------------------------------------|---------------------------------------------------------|
| 13       | 0                          | 1.9      | 14.3                                                       | 1.8                                                     |
| 14       | 5                          | 2.0      | 15.8                                                       | 2.0                                                     |
| 15       | 10                         | 2.0      | 17.5                                                       | 2.4                                                     |

A photographic film was prepared in the same manner as in Example 1 to measure the water escape rate. Thus, with photographic Films No. 13, 14 and 15, 11 days, less than 11 days and 10 days, respectively, were required for water to escape as a vapor. The flatness of the surfaces of the photographic pictures did not change upon escape of water, and photographic films capable of being stored for a long period of time were obtained.

## EXAMPLE 5

Subbing layers of a thickness of 0.3 $\mu$  were provided on both sides of the biaxially oriented polyester film base having a thickness of 150 $\mu$  as described in Example 1, and a backing layer of cellulose diacetate of a thickness of 10 $\mu$  was provided on the back side. Then, the

following photographic layers were coated in sequence to complete a light-sensitive element.

## (1) Image-Receiving Layer

5 A layer comprising 3 g/m<sup>2</sup> of a mordant of copoly(styrenevinyl benzene-tri-n-hexylbenzylammonium chloride) and 3 g/m<sup>2</sup> of gelatin.

## (2) Light-Reflecting Layer

10 A layer comprising 20 g/m<sup>2</sup> of titanium dioxide and 2 g/m<sup>2</sup> of gelatin.

## (3) Light-Intercepting Layer

15 A layer comprising 2.7 g/m<sup>2</sup> of carbon black and 2.7 g/m<sup>2</sup> of gelatin.

## (4) Cyan Color Image-Providing Material Layer

A layer containing 0.5 g/m<sup>2</sup> of a cyan color image-providing compound, Compound (P), 0.25 g/m<sup>2</sup> of N,N-diethyllaurylamide and 1.14 g/m<sup>2</sup> of gelatin.

## (5) Red-Sensitive Internal Latent Image Forming Type Emulsion Layer

25 A layer containing silver bromide (1.9 g silver/m<sup>2</sup>), 28 mg/m<sup>2</sup> of a fogging agent, Compound (S), 0.14 g/m<sup>2</sup> of sodium pentadecylhydroquinonesulfonate, and 1.4 g/m<sup>2</sup> of gelatin.

## (6) Interlayer

30 A layer comprising 0.8 g/m<sup>2</sup> of 2,5-di-tert-pentadecylhydroquinone and 2.6 g/m<sup>2</sup> of gelatin.

## (7) Magenta Color Image-Providing Material Layer

35 A layer containing 0.45 g/m<sup>2</sup> of a magenta color image-providing compound, Compound (Q), 0.10 g/m<sup>2</sup> of N,N-diethyllaurylamide and 1.1 g/m<sup>2</sup> of gelatin.

## (8) Green-Sensitive Internal Latent Image Forming Type Emulsion Layer

40 A layer containing 28 mg/m<sup>2</sup> of a fogging agent, Compound (S), 0.14 g/m<sup>2</sup> of sodium pentadecylhydroquinonesulfonate and 1.4 g/m<sup>2</sup> of gelatin.

## (9) Interlayer

45 A layer comprising 0.8 g/m<sup>2</sup> of 2,5-di-tert-pentadecylhydroquinone and 2.6 g/m<sup>2</sup> of gelatin.

## (10) Yellow Color-Providing Material Layer

50 A layer containing 0.8 g/m<sup>2</sup> of a yellow color image-providing compound, Compound (R), 0.16 g/m<sup>2</sup> of N,N-diethyllaurylamide and 0.8 g/m<sup>2</sup> of gelatin.

## (11) Blue-Sensitive Internal Latent Image Forming Type Emulsion Layer

A layer containing silver bromide (1.9 g silver/m<sup>2</sup>), 28 mg/m<sup>2</sup> of a fogging agent, 0.14 g/m<sup>2</sup> of sodium pentadecylhydroquinonesulfonate and 1.4 g/m<sup>2</sup> of gelatin.

## (12) Protective Layer

A layer comprising 0.9 g/m<sup>2</sup> of gelatin. These photographic layers were hardened with 1,3-bisvinylsulfonyl-2-propanol.

The compounds used in preparing the above layers had the following formulas.

Compound (P)

-continued



Subbing layers having a thickness of  $0.3\mu$  were provided on both sides of a biaxially oriented film base of a thickness of  $100\mu$  of the polyester described in Example 1, and a backing layer comprising cellulose diacetate having a thickness of  $7\mu$  was provided on the back side. Then, the following photographic layers were coated in sequence to complete a cover sheet.

#### (1) Polymer Acid Layer

A layer comprising  $25\text{ g/m}^2$  of an n-butylacrylic acid-acrylic acid copolymer (mol. wt.: about 70,000; 3:7 wt. ratio).

#### (2) Neutralization Timing Layer

A layer comprising  $3.8\text{ g/m}^2$  of cellulose acetate (acetylation degree: 39.4%) and  $0.2\text{ g/m}^2$  of copoly(styrene-maleic anhydride).

Further, a processing solution having the following composition was prepared and sealed in a pod.

|    |                                                  |      |   |
|----|--------------------------------------------------|------|---|
| 10 | 1-Phenyl-4-methyl-4-hydroxymethyl-3-pyrazolidine | 10   | g |
|    | Methylhydroquinone                               | 0.18 | g |
|    | 5-Methylbenzotriazole                            | 4.0  | g |
|    | Sodium Sulfite (anhydrous)                       | 1.0  | g |
|    | Sodium Carboxymethyl Cellulose                   | 40   | g |
| 15 | Carbon Black                                     | 150  | g |
|    | Potassium Hydroxide                              | 50   | g |
|    | Water                                            | 550  | g |

The thus-prepared light-sensitive sheet, the cover sheet and the processing solution-retaining pod were disposed as described in U.S. Pat. No. 4,042,395 to prepare a film unit. That is, in order to ensure a space of a thickness of  $125\mu$  between the light-sensitive sheet in a rectangular form and the cover sheet, polyester strips were heat-sealed to one pair of opposing sides of the light-sensitive sheet and the cover sheet, and the processing solution-retaining pod and an excess solution reservoir were fixedly positioned at each of the other pair of opposing ends.

This film unit was subjected to color photographic sensitometry through the cover sheet, and passed between a pair of pressure-applying metal rollers to spread the processing solution in a solution thickness of about  $100\mu$  between the light-sensitive sheet and the cover sheet. A color image with good color separation was formed about 10 minutes after spreading the processing solution.

A corresponding comparative film unit was prepared under the same conditions as described above except for using a conventional biaxially oriented polyethylene terephthalate film of the same thickness as a film base, and processed in the same manner. Thus, a color image with as good a color separation as that of the above-described film unit was obtained.

These film units were left under the conditions of  $20^\circ\text{C}$ . and 65% RH, and the amount of water escape as vapor from the film unit was determined by measuring the weight loss. Thus, it was found that, with the film unit of the present invention and the comparative film unit using a conventional type polyester film base, it took 10 days and about 28 days, respectively, for water in the processing solution to escape as vapor. These two film units showed good flatness during processing and storage.

Another two pairs of the film units similarly prepared and processed were subjected to color image-fading testing on and after the third day from their processings to obtain the following results.

TABLE 4

| Sample                     | Fading Test                | Fading Degree (3) |           |           |
|----------------------------|----------------------------|-------------------|-----------|-----------|
|                            |                            | B Density         | G Density | R Density |
| Film Unit of the Invention | Fading with Light (1)      | -0.08             | -0.05     | -0.35     |
|                            | Fading in a Dark Place (2) | -0.03             | -0.10     | +0.02     |
| Film Unit for Comparison   | Fading with Light (1)      | -0.10             | -0.25     | -0.50     |
|                            | Fading in a                | -0.08             | -0.25     | +0.05     |

TABLE 4-continued

| Sample         | Fading Test | Fading Degree (3) |           |           |
|----------------|-------------|-------------------|-----------|-----------|
|                |             | B Density         | G Density | R Density |
| Dark Place (2) |             |                   |           |           |

(1) Conditions of fading with light: irradiation with light of about 15,000 lux emitted from a day-light fluorescent lamp at about 35° C. for 7 days.

(2) Conditions for fading in a dark place: storage for 14 days in a well-circulated air thermostatically controlled chamber at 60° C. and 60% RH.

(3) Difference in density occurring on test based on an initial density of 1.5.

The above results clearly show that the film unit of the present invention can be rapidly dried after processing while maintaining good flatness and that the color images formed therein are fast and undergo less change in density.

While the invention has been described in detail and with reference to specific embodiments thereof, it will be apparent to one skilled in the art that various changes and modifications can be made therein without departing from the spirit and scope thereof.

What is claimed is:

1. A diffusion transfer photographic film which comprises a support, a silver halide layer and an image receiving layer, in which a film of a polyethylene terephthalate copolymer is a part of the constituents thereof, said polyethylene terephthalate copolymer containing about 3 to about 20% by weight of a polyalkylene glycol having a molecular weight of about 300 to about 30,000, as a glycol component comonomer, based on the weight of the polyethylene terephthalate copolymer.

2. The diffusion transfer photographic film as described in claim 1, wherein said polyalkylene glycol is present in a copolymerization ratio of 3 to 15% by weight.

3. The diffusion transfer photographic film as described in claim 1, wherein said polyalkylene glycol has a molecular weight of about 800 to about 20,000.

4. The diffusion transfer photographic film as described in claim 2, wherein said polyalkylene glycol has a molecular weight of about 800 to about 20,000.

5. The diffusion transfer photographic film as described in claim 1, wherein said polyalkylene glycol is selected from the group consisting of polyethylene glycol, polypropylene glycol, poly(ethylene-propylene)-glycol copolymer and polytetramethylene glycol.

6. The diffusion transfer photographic film as described in claim 5, wherein said polyalkylene glycol is polyethylene glycol and the polyethylene glycol is present in a copolymerization ratio of 4 to 10% by weight.

7. The diffusion transfer photographic film as described in claim 6, wherein said polyethylene glycol has a molecular weight of about 300 to about 10,000.

8. The diffusion transfer photographic film as described in claim 7, wherein said polyethylene glycol has a molecular weight of about 800 to about 6,000.

9. The diffusion transfer photographic film as described in claim 8, wherein said polyethylene glycol has a molecular weight of about 800 to about 2,000.

10. The diffusion transfer photographic film as described in claim 2, wherein said polyalkylene glycol is selected from the group consisting of polyethylene glycol, polypropylene glycol, poly(ethylene-propylene) glycol copolymer and polytetramethylene glycol.

11. The diffusion transfer photographic film as described in claim 8, wherein said polyalkylene glycol is polyethylene glycol and the polyethylene glycol is present in a copolymerization ratio of 4 to 10% by weight.

12. The diffusion transfer photographic film as described in claim 11, wherein said polyethylene glycol has a molecular weight of about 300 to about 10,000.

13. The diffusion transfer photographic film as described in claim 12, wherein said polyethylene glycol has a molecular weight of about 800 to about 6,000.

14. The diffusion transfer photographic film as described in claim 13, wherein said polyethylene glycol has a molecular weight of about 800 to about 2,000.

15. The diffusion transfer photographic film as described in claim 1, wherein said film of a polyethylene terephthalate copolymer contains an antioxidant.

16. The diffusion transfer photographic film as described in claim 13, wherein said antioxidant is a hindered phenol compound.

17. The diffusion transfer photographic film as described in claim 1, wherein a film of said polyethylene terephthalate copolymer is a biaxially oriented film of said polyethylene terephthalate copolymer.

18. The diffusion transfer photographic film as described in claim 1, wherein said film of a polyethylene terephthalate copolymer has a water vapor permeability at 40° C. of about 10 to 100 g/m<sup>2</sup>·24 hr/0.1 mm and a humidity swelling coefficient at 20° C. of about 1.0×10<sup>-5</sup> to 6.0×10<sup>-5</sup>/% RH.

19. A composite diffusion transfer unit adapted for use in a photographic diffusion transfer process comprising two dimensionally stable supports at least one of which is transparent having sandwiched therebetween at least:

(i) at least one light-sensitive silver halide emulsion layer;

(ii) at least one dye image-forming compound associated with each of said at least one silver halide emulsion layer and capable of image-wise forming a diffusible dye as a result of the development of said at least one silver halide emulsion layer;

(iii) an image-receiving layer capable of fixing the image-wise formed diffusible dye as a photographic image; and

(iv) a light-reflecting layer forming a background for viewing the image formed in said image-receiving layer and a container retaining an aqueous alkaline processing solution to be spread between said supports, and wherein at least one of said dimensionally stable supports comprises a film of a polyethylene terephthalate copolymer containing about 3 to about 20% by weight of a polyalkylene glycol having a molecular weight of about 300 to about 30,000, as a glycol component comonomer, based on the weight of the polyethylene terephthalate copolymer.

20. The film unit as described in claim 19, wherein said film unit has a structure such that part of said dimensionally stable supports does not substantially come into contact with said aqueous processing solution even after said aqueous processing solution has been spread.

21. The film unit as described in claim 20, which has a structure such that at least part of the periphery of said dimensionally stable supports is strongly secured with a member which is not substantially swollen when in contact with said aqueous processing solution.

22. A composite diffusion transfer photographic film unit adapted for use in a photographic diffusion transfer process comprising:

- (a) a photosensitive element comprising a dimensionally stable transparent support having thereon the following layers in sequence: an image-receiving layer; an alkaline solution-permeable, light-reflecting layer; an alkaline solution-permeable opaque layer; a red-sensitive silver halide emulsion layer having a cyan dye image-providing compound associated therewith; an interlayer; a green-sensitive silver halide emulsion layer having a magenta dye image-providing compound associated therewith; an interlayer; a red-sensitive silver halide emulsion layer having a yellow dye image-providing compound associated therewith; and a protective layer;
- (b) a cover sheet superposed on said protective layer of said photosensitive element and comprising a dimensionally stable transparent support coated in sequence with a neutralizing layer and a neutralization timing layer; and
- (c) a rupturable container retaining an aqueous alkaline processing composition and an opacifying agent, said rupturable container being so positioned during the processing of said film unit that a compressive force applied to said rupturable container causes a discharge of said alkaline processing composition between said cover sheet and said protective layer of said photosensitive element, wherein at least one of said dimensionally stable transparent supports comprises a film of a polyethylene terephthalate copolymer containing about 3 to about 20% by weight of a polyalkylene glycol having a molecular weight of about 300 to about 30,000, as a glycol component comonomer, based on the weight of the polyethylene terephthalate copolymer.

23. The film unit as described in claim 22, wherein both said support of said photosensitive element and said support of said cover sheet are a film of said polyethylene terephthalate copolymer.

24. The film unit as described in claim 22, wherein said polyalkylene glycol has a molecular weight of about 800 to about 20,000.

25. The film unit as described in claim 24, wherein said polyalkylene glycol is present in a copolymerization ratio of 3 to 15% by weight.

26. The film unit as described in claim 25, wherein said film of a polyethylene terephthalate copolymer is a biaxially oriented film of said polyethylene terephthalate copolymer.

27. The film unit as described in claim 26, wherein said film of a polyethylene terephthalate copolymer has a water vapor permeability at 40° C. of about 10 to 100 g/m<sup>2</sup> 24 hr/0.1 mm and a humidity swelling coefficient at 20° C. of about  $1.0 \times 10^{-5}$  to  $6.0 \times 10^{-5}$  % RH.

28. In a cover sheet for use with a color diffusion transfer unit, which comprises a transparent support having coated thereon, in sequence, a neutralizing layer and a neutralization timing layer, the improvement

which comprises said transparent support comprising a film of a polyethylene glycol having a molecular weight of about 300 to about 30,000, as a glycol component comonomer, based on the weight of the polyethylene terephthalate copolymer.

29. In a process of producing a photographic diffusion transfer image, comprising image-wise exposing the film unit as described in claim 19 and discharging said aqueous processing solution between said two supports.

30. A process of producing a photographic diffusion transfer image, comprising image-wise exposing a film unit as below described and discharging an aqueous processing solution between said two dimensionally stable transparent supports as below described wherein said film unit comprises:

- (a) a photosensitive element comprising a dimensionally stable transparent support having thereon the following layers in sequence: an image-receiving layer; an alkaline solution-permeable, light-reflecting layer; an alkaline solution-permeable opaque layer; a red-sensitive silver halide emulsion layer having a cyan dye image-providing compound associated therewith; an interlayer; a green-sensitive silver halide emulsion layer having a magenta dye image-providing compound associated therewith; an interlayer; a red-sensitive silver halide emulsion layer having a yellow dye image-providing compound associated therewith; and a protective layer;
- (b) a cover sheet superposed on said protective layer of said photosensitive element and comprising a dimensionally stable transparent support coated in sequence with a neutralizing layer and a neutralization timing layer; and
- (c) a rupturable container retaining an aqueous alkaline processing composition and an opacifying agent, said rupturable container being so positioned during the processing of said film unit that a compressive force applied to said rupturable container causes a discharge of said alkaline processing composition between said cover sheet and said protective layer of said photosensitive element;

wherein said image-wise exposing is through said cover sheet and wherein at least one of said dimensionally stable transparent supports comprises a film of a polyethylene terephthalate copolymer containing about 3 to about 20% by weight of a polyalkylene glycol having a molecular weight of about 300 to about 30,000, as a glycol component comonomer, based on the weight of the polyethylene terephthalate copolymer.

31. In a photographic element comprising a support, at least one silver halide emulsion layer having associated therewith a dye image-providing compound, an image receiving layer and a neutralizing layer, said element containing a neutralization timing layer between said neutralizing layer and said silver halide emulsion layer, the improvement comprising said support is a film of a polyethylene terephthalate copolymer containing about 3 to 20% by weight of a polyalkylene glycol having a molecular weight of about 300 to about 30,000, as a glycol component comonomer, based on the weight of the polyethylene terephthalate copolymer.

\* \* \* \* \*